

July 21, 1953

J. W. HUTCHESON ET AL  
MANUFACTURE OF ZINC SALTS OF HIGH MOLECULAR  
WEIGHT ALKYLATED HYDROXY AROMATIC COMPOUNDS  
Filed Feb. 11, 1950

2,646,402



LUBRICATING OIL CONCENTRATE OF Zn ALKYL PHENOLATE BY

INVENTORS  
JOHN W. HUTCHESON  
EDWIN C. KNOWLES

*John W. Hutcheson*

*J. C. Knowles*

ATTORNEYS

Patented July 21, 1953

2,646,402

UNITED STATES PATENT OFFICE

2,646,402

MANUFACTURE OF ZINC SALTS OF HIGH  
MOLECULAR WEIGHT ALKYLATED HY-  
DROXY AROMATIC COMPOUNDS

John W. Hutcheson, Beacon, and Edwin C.  
Knowles, Glenham, N. Y., assignors to The  
Texas Company, New York, N. Y., a corporation  
of Delaware

Application February 11, 1950, Serial No. 143,762

4 Claims. (Cl. 252—42.7)

1

This invention relates to the manufacture of zinc salts of high molecular weight alkylated hydroxy aromatic compounds, such as alkyl phenols, wherein the substituent alkyl group on each benzene nucleus contains from 15 to 30 carbon atoms.

The zinc salts of alkylated hydroxy aromatic compounds, such as alkyl phenols, having one or more high molecular weight alkyl side chains substituted on the ring, are valuable additives for mineral lubricating oil. The zinc alkyl phenolate of the present invention is particularly useful, when used in conjunction with a magnesium alkyl phenolate, as an additive for an airplane engine oil of the highly refined residual type, as disclosed and claimed in the copending application of Frederic C. McCoy, Bill L. Benge, Edwin C. Knowles, and Charles C. Towne, Serial No. 286,634 filed May 7, 1952, as a continuation-in part of Serial No. 143,836, February 11, 1950, now abandoned.

It is known to prepare polyvalent metal salts of lower molecular weight alkyl phenols or other alkylated hydroxy aromatic hydrocarbons by a double decomposition procedure, involving first forming the alkali metal salt of the alkyl phenol, followed by a reaction with a soluble polyvalent metal salt, such as a chloride. It has been found that the conventional procedure of carrying out this double decomposition reaction is unsatisfactory in the preparation of the zinc salts of high molecular weight alkylated hydroxy aromatic hydrocarbons, such as alkyl phenols, wherein the substituent alkyl group of the benzene nucleus contains from 15 to 30 carbon atoms, since the quality of the final product is unsatisfactory with respect to solubility and effectiveness as a residual mineral lubricating oil additive.

It is accordingly a principal object of the present invention to provide an improved process of synthesizing the zinc salts of higher molecular weight alkylated hydroxy aromatic hydrocarbons, such as alkyl phenols, wherein the substituent alkyl group of the benzene nucleus contains from 15 to 30 carbon atoms, in order to provide products of the required solubility and quality to serve as lubricating oil additives, particularly of the residual lubricating oil type.

Other objects and advantages of the present invention will be apparent from the following description taken in conjunction with the attached drawing and appended claims.

The drawing is a flow sheet of the method of synthesis of a preferred zinc alkyl phenolate in accordance with the present invention.

Any suitable alkylated hydroxy aromatic hydrocarbon, wherein the substituent alkyl group on the benzene nucleus contains from 15 to 30 carbon atoms, is a satisfactory starting material for purposes of the present invention. The preferred material from the standpoint of additive

manufacture is an alkyl phenol prepared by alkylating a mononuclear monohydroxy aromatic hydrocarbon, such as phenol, cresol or other alkyl phenol, with an olefin polymer, such as a propylene polymer, containing from about 16 to 30 carbon atoms. Also hydrogenated cardanol producing a C<sub>15</sub> alkyl phenol is a satisfactory starting material. Likewise, alkylated mononuclear polyhydroxy aromatic hydrocarbons, such as hydroquinone, pyrogallol and other dihydric and trihydric phenols, can be employed. Also, alkylated polynuclear hydroxy aromatic hydrocarbons, such as the naphthols, can be used. From the standpoints of availability and economy, alkyl phenol prepared by alkylating phenol with a C<sub>18</sub>—C<sub>30</sub>, and preferably C<sub>18</sub>—C<sub>28</sub>, propylene polymer in the presence of anhydrous HF catalyst as disclosed and claimed in the copending application of Louis B. Bos Serial No. 143,784 filed of even date herewith, or in the presence of AlCl<sub>3</sub>·HSO<sub>4</sub> complex catalyst as disclosed and claimed in the copending application of Fred W. Moore and Herman D. Kluge Serial No. 143,782, filed of even date herewith, is preferred. For the purpose of ease in description, a C<sub>15</sub>—C<sub>30</sub> alkyl phenol of the foregoing type will be referred to in the following text; but it is to be understood that this is solely by way of example, and that the description applies to the other alkylated hydroxy aromatic hydrocarbons specified.

The synthesis of the zinc salt of a C<sub>15</sub>—C<sub>30</sub> alkyl phenol in accordance with the present invention involves an improvement on the known double decomposition reaction procedure, wherein the alkyl phenol is reacted with an alkali metal alcoholate, generally sodium butylate, and the resulting sodium alkyl phenolate is reacted with a soluble zinc salt, such as the acetate, to form the zinc alkyl phenolate. The double decomposition reaction between the sodium alkyl phenolate and zinc acetate is represented by the following equation:



The improvement features of the present invention involve the following. Anhydrous conditions are maintained throughout the reaction and recovery of the product. Substantially equal molar amounts of the alkyl phenol and the alkali metal butylate or other alcoholate, in solution in an excess of the corresponding anhydrous aliphatic alcohol, are reacted with the soluble zinc salt at an elevated temperature providing alcohol

refluxing conditions for a reaction time in excess of 20 hours and up to 48 hours, preferably about 24 hours. In this reaction, the sodium butylate or other alcoholate in solution in a portion of the total anhydrous aliphatic alcohol is added slowly or dropwise to a premixture of the alkyl phenol and the zinc salt in the balance of the anhydrous alcohol at a lower temperature of the order of 30-70° C., preferably about 50° C.; and then the temperature of the resulting mix is raised to the alcohol refluxing temperature and maintained at this temperature for the stated long reaction time. A slight excess over the stoichiometric equivalent of  $\frac{1}{2}$  molar amount based on the other reactants of the zinc salt is employed in the reaction. A mineral lubricating oil, which forms a concentrate of the final zinc alkyl phenolate in the oil, is added only after completion of the reaction and filtration of the reaction mix to remove the precipitated alkali metal salt. A light hydrocarbon solvent, such as pentane, is added to the mineral lubricating oil concentrate of the zinc alkyl phenolate, and the resulting mix refiltered, followed by stripping of the hydrocarbon solvent, to obtain a purified concentrate as the desired final product. The foregoing features have been found critical in producing a zinc alkyl phenolate of the required solubility and quality for use as an additive in residual mineral lubricating oil of the airplane engine oil type.

Referring to the drawing, the essential starting materials are illustrated for the preferred example as sodium metal, anhydrous butyl alcohol, a C<sub>15</sub>-C<sub>30</sub> alkyl phenol and zinc acetate. In place of anhydrous butyl alcohol, other anhydrous aliphatic alcohols boiling above the boiling point of water, selected from the group of C<sub>4</sub> to C<sub>6</sub> aliphatic alcohols can be employed. In place of the zinc acetate, other zinc carboxylate or inorganic salts, the acidic portion of which forms an alkali metal salt which is insoluble in the anhydrous aliphatic alcohol, such as the formate, butyrate, chloride, etc., can be used. Also, other alkali metals, such as potassium, can be employed. It will be understood that the reactants illustrated are preferred.

An important feature of the present invention is the provision of substantially anhydrous reactants and the maintenance of anhydrous conditions throughout the synthesis. For this purpose, the sodium metal is maintained submerged in a suitable liquid, such as toluene, which is inert to the metal; and the metal is cut or subdivided in small pieces for the reaction while submerged in the liquid. The butyl alcohol is dried by distillation before being used; and the zinc salt is carefully heated to fusion to be sure that it is anhydrous. In the case of zinc chloride, this can also be dried by refluxing in the presence of toluene. The alkyl phenol and the zinc acetate or other zinc salt are charged in the ratio of one molar quantity of the alkyl phenol to slightly more than  $\frac{1}{2}$  molar quantity of the zinc salt, together with a portion of the anhydrous butyl alcohol, to a stirred reactor fitted with a condenser for refluxing, and provided with drying tubes on all openings to the atmosphere. In a separate vessel, the freshly cut sodium metal, which has been protected from the atmosphere by submergence as previously described, is mixed with the balance of the anhydrous butyl alcohol to form a sodium butylate solution in excess anhydrous butyl alcohol.

The sodium butylate (Reactant No. 1) in the

butyl alcohol is then added slowly or dropwise in the proportion of one molar amount to the premixture of the alkyl phenol (Reactant No. 2) and the zinc acetate (Reactant No. 3) in solution in the balance of the alcohol at a temperature of about 30-70° C., preferably about 50° C., while the contents of the reactor are stirred. This has been found important in producing precipitated sodium acetate crystals of larger size which can be properly filtered from the reaction mix. Moreover, all openings from the reactor to the atmosphere are fitted with drying tubes to protect the reactants from atmospheric moisture and maintain the anhydrous conditions. Following the addition of the sodium butylate solution, the reactor is then heated to a butyl alcohol reflux temperature and maintained at that temperature with continued stirring for a reaction period in excess of 20 hours, preferably about 24 hours. This long reaction period has been found important in producing a zinc alkyl phenolate of the desired quality for purposes of the present invention.

The resulting reaction mix while hot is then filtered, preferably through a layer of dried solid filter-aid material such as "Super Cel Hy-Flo," to remove the precipitated sodium acetate. The resulting filtrate of zinc alkyl phenolate in solution in anhydrous butyl alcohol is then mixed with sufficient dry mineral lubricating oil, such as a refined paraffin base distillate motor oil of about SAE 10 grade, or a refined naphthene base oil having an SUS viscosity at 100° F. of about 300, to produce an ultimate concentrate of the zinc alkyl phenolate in the lubricating oil of about 10-60%, preferably about 50%. The butyl alcohol is then stripped from the lubricating oil concentrate by distillation with the aid of a dry gas, such as dry air.

In order to effect further purification of the concentrate and improve the quality of the zinc alkyl phenolate product as a lubricating oil additive, the concentrate is then mixed with a light hydrocarbon solvent which is also anhydrous, such as dry pentane, hexane or light gasoline. A volume of the light hydrocarbon solvent equivalent to about  $\frac{1}{2}$  to twice the volume of the concentrate, preferably about an equal volume, is employed for this purpose. As shown, dry pentane is preferred as the hydrocarbon solvent. The resulting solution is then refiltered while hot in the manner described above for the first filtration. The pentane or other hydrocarbon solvent is then stripped by distillation with the aid of dry air to obtain the purified concentrate of zinc alkyl phenolate as the final product.

The following examples are given to further illustrate the present invention:

#### EXAMPLE 1

1284 grams of alkyl phenol (3 mols), wherein the substituent alkyl group on the benzene nucleus contained an average of 24 carbon atoms, together with 300 grams of fused C. P. zinc acetate (1.5 mols + 25 grams, were mixed with 305 grams of a naphthene base distillate lubricating oil having an SUS viscosity at 100° F. of 315, and about half of 2,000 grams of anhydrous butyl alcohol. The mixture was charged to a flask fitted with a stirrer and condenser and heated to 150° F. In a separate flask, 69 grams (3 mols) of sodium metal were reacted with the balance of the butyl alcohol. The resulting sodium butylate solution in excess butyl alcohol was then added to the other reactants, and the materials heated

## 5

and held at butyl alcohol reflux for seven hours. After standing overnight, the material was filtered through "Super Cel Hy-Flo," the solvent then stripped, and the lubricating oil concentrate refiltered. Considerable foaming was experienced during the refluxing which required the use of an anti-foam agent to control, and difficulty was experienced in the filtrations. A yield of 2,070 grams of a lubricating oil concentrate of zinc alkyl phenolate was secured, which analyzed to an ash content of 4.68% basis a theoretical ash content of 4.4%, and a zinc content of 3.67% basis a theoretical zinc content of 3.56%. The material was soluble in a distillate paraffin base motor oil of SAE 10 grade to the extent of dissolving 1% of the zinc alkyl phenolate therein, and the resulting solution remained clear on storage at a temperature of 120° F.

A second batch of zinc alkyl phenolate concentrate, employing the same quantities of materials and the same procedure as above set forth except that a reaction time under refluxing conditions of 20 hours was used, yielded 1950 grams of a concentrate which also analyzed somewhat high in ash and zinc contents based on theoretical. These two batches of concentrate were combined for engine testing. While the products appeared satisfactory on the basis of their ash and zinc contents and solubility in distillate lubricating oil, the results of the engine test were not satisfactory as described in greater detail hereinbelow.

## EXAMPLE 2

In this case zinc chloride was employed as the zinc salt, the materials employed being as follows:

|                              |                              |
|------------------------------|------------------------------|
| C <sub>22</sub> alkyl phenol | 208 grams (1/2 mol)          |
| Sodium metal                 | 11.5 grams (1/2 mol)         |
| Zinc chloride CP             | 40 grams (1/4 mol + 6 grams) |
| Butyl alcohol                | 500 mls.                     |
| Naphthene base distillate    |                              |
| lubricating oil              | 224 grams                    |

The same procedure was employed as in the foregoing Example 1 except that the zinc chloride was added to the alkyl phenol, the naphthene base lubricating oil and part of the butyl alcohol at a temperature of 70° C., and this temperature maintained for 1½ hours prior to the addition of the sodium butylate solution in the remaining butyl alcohol. Following the rapid addition of the sodium butylate solution, the reactants were heated at butyl alcohol reflux for 20 hours. A yield of 405 grams of concentrate which analyzed to an ash content of 4.37% basis a theoretical 4.54%, and a zinc content of 3.50% basis a theoretical 3.63%, was obtained. The material was soluble in a refined residual lubricating oil of the airplane engine oil type to the extent of dissolving 1% of the zinc alkyl phenolate in the oil, the solution remaining clear for five months storage at 120° F. While the product appeared satisfactory basis the ash and zinc contents as well as its solubility and storage properties, the results of engine testing showed the product to be unsatisfactory from the standpoint of maintaining desired engine cleanliness as discussed hereinbelow. The residual lubricating oil of the airplane engine oil type was refined by solvent disasphalting, solvent refining, solvent dewaxing, clay contacting and clay filtering. Airplane engine oils of this type generally have an SUS viscosity at 210° F. at about 80-130. The particular oil selected for the above described storage test had an SUS viscosity at 210° F. of about 120.

## 6

## EXAMPLE 3

The materials employed were:

|                              |                               |
|------------------------------|-------------------------------|
| C <sub>22</sub> alkyl phenol | 388 grams (1 mol)             |
| Sodium metal                 | 23 grams (1 mol)              |
| Zinc acetate CP fused        | 100 grams (1/2 mol + 8 grams) |
| Butyl alcohol                | 800 mls.                      |
| Naphthene base distillate    |                               |
| lubricating oil              | 419 grams                     |

The procedure employed was similar to Example 1 above, except that the sodium butylate solution was added dropwise to the other reactants at a temperature of 50° C., and then the temperature of the resulting mix was increased gradually to butyl alcohol reflux and maintained at a reflux temperature for 20 hours. A yield of 633 grams of a concentrate analyzing to an ash content of 3.57% basis a theoretical of 4.82% and a zinc content of 2.19% basis a theoretical of 3.87%, was obtained. The material was soluble in the residual airplane engine oil of 120 grade to the extent of 1% of the pure zinc alkyl phenolate when initially prepared, but a slight precipitate developed in one month storage both at 120° F. and at room temperature. While the material did not appear particularly promising from the standpoints of low ash and zinc contents and poor stability on storage, it was nevertheless engine tested; but the engine test results were not satisfactory as set forth hereinbelow.

## EXAMPLE 4

The same procedure as in Example 3 was employed except that a 10% excess quantity of alkyl phenol was present in the reacting mix. Quantities of materials employed were as follows:

|                              |                               |
|------------------------------|-------------------------------|
| C <sub>22</sub> alkyl phenol | 915 grams (2 mols + 83 grams) |
| Sodium metal                 | 46 grams (2 mols)             |
| Zinc acetate CP fused        | 200 grams (1 mol + 17 grams)  |
| Butyl alcohol                | 1500 mls.                     |
| Naphthene base distillate    |                               |
| lubricating oil              | 875 grams                     |

A yield was obtained of 1604 grams of concentrate analyzing 4.86% ash based on a theoretical of 4.52% and 3.03% zinc based on a theoretical of 3.50. The material was soluble in the residual airplane engine oil of 120 grade to the extent of dissolving 1% of the zinc alkyl phenolate therein when freshly prepared; but a precipitate formed on storage at both 120° F. and room temperature in one month. The product was engine tested, but the results were not satisfactory as pointed out hereinbelow.

## EXAMPLE 5

The materials employed were:

|                              |                                    |
|------------------------------|------------------------------------|
| C <sub>22</sub> alkyl phenol | 1688 grams (4 mols)                |
| Sodium metal                 | 92 grams (4 mols)                  |
| Zinc acetate CP fused        | 400 grams (2 mols + 32 grams)      |
| Butyl alcohol (dry)          | 3000 mls.                          |
| Naphthene base distillate    |                                    |
| lubricating oil              | Sufficient to make 50% concentrate |

In this preparation, precautions were taken to maintain absolutely anhydrous conditions. The butyl alcohol was dried by distillation before use. The sodium metal was maintained and cut under toluene. The naphthene base lubricating oil was not added until the reaction had been completed, the precipitated sodium acetate filtered and a portion of the butyl alcohol stripped from the filtrate. The procedure was otherwise the same as for Example 3, except that refluxing conditions during the reaction were maintained for 30 hours for a portion of the sample and for 48 hours for the balance of the sample. A total yield of 2830 grams of a 50% concen-

trate was obtained. The tests on the sample which had been refluxed for 30 hours are typical, with an ash content of 4.21 based on a theoretical of 4.46%, and a zinc content of 2.63 based on a theoretical of 3.58%. The material was soluble to the extent of dissolving at least 1% of the zinc alkyl phenolate in the residual airplane engine oil of 120 grade, and had excellent stability as evidenced by the solution remaining clear for two months storage at 120° F. and also at room temperature. The product was employed in engine testing with greatly improved results in comparison to the tests on the products of the previous examples, as pointed out hereinbelow.

## EXAMPLE 6

Based on the foregoing results including the engine tests, a so-called standard procedure was developed in accordance with the following example. The materials employed were:

C<sub>22</sub> alkyl phenol..... 844 grams (2 mols)  
Sodium metal..... 46 grams (2 mols)  
Zinc acetate CP fused..... 200 grams (1 mol + 17 grams)  
Butyl alcohol (dry)..... 2,500 mls.  
Naphthalene base distillate lubricating oil..... 900 grams

The butyl alcohol was dried by distillation before use. The sodium metal was maintained and cut under toluene. All open condensers and flasks were protected from moisture in the atmosphere by the use of drying tubes. All stripping was carried out by the use of dry air.

The alkyl phenol, zinc acetate and a portion of the dry butyl alcohol were charged to the reactor and the reactants heated to 50° C. The sodium was reacted in a separate vessel with remaining dry butyl alcohol. The sodium butylate solution was then added dropwise to the other reactants at 50° C. Following the addition of the sodium butylate solution, the temperature was gradually increased to butyl alcohol reflux and this was maintained for 24 hours. The reaction mix was then filtered and the naphthalene base distillate lubricating oil, which was sufficient to make a 50% concentrate, was added to the filtrate. The butyl alcohol was then stripped with the aid of dry air. After stripping, the product was dissolved in about an equal volume of dry pentane, refiltered and the pentane removed by stripping with dry air.

A yield was obtained of 1038 grams of concentrate, analyzing 2.96% ash with a theoretical of 4.46%, and 1.95% zinc with a theoretical of 3.58%. While the products prepared by this standard procedure generally have low ash and zinc contents as illustrated by the foregoing, this appears to be characteristic of entirely satisfactory zinc alkyl phenolate preparations for purposes of the present invention. Thus this product was satisfactorily soluble to the extent of 1% of the zinc alkyl phenolate in the residual airplane

engine oil, and had excellent stability with the solution remaining clear for two months storage at 120° F. and at room temperature. The product was employed in engine testing with excellent results as set forth hereinbelow.

As set forth more fully in the above-mentioned copending application of Frederic C. McCoy, Bill L. Benge, Edwin C. Knowles, and Charles C. Towne, the zinc alkyl phenolate produced in accordance with the present invention is employed in conjunction with a second alkyl phenolate, namely magnesium alkyl phenolate, in an airplane engine oil, to maintain engine cleanliness in high temperature heavy duty service, and also to prevent the formation of objectionable combustion chamber deposits. Final proof of the quality of the zinc alkyl phenolate preparation was therefore secured by the actual engine testing of the preparation in conjunction with a magnesium alkyl phenolate of known satisfactory quality in an airplane engine oil, as set forth in the following table. In that table, ZP designates zinc alkyl phenolate, MP designates magnesium alkyl phenolate, and the numeral following the designation for these metallic phenolates signifies the average carbon atom content of the alkyl side chain on each benzene nucleus of the salt.

The CFR High Speed Engine Test of the table is recognized as a reliable screening test for determining the ability of a crank case lubricating oil to reduce engine deposits under severe operating conditions. This test is carried out with a standard CFR single cylinder engine operating under the following conditions:

|                            |                                                               |
|----------------------------|---------------------------------------------------------------|
| 35. Compression ratio..... | 6.5:1                                                         |
| Speed, R. P. M.....        | 1,800                                                         |
| Air/fuel ratio.....        | 13:1                                                          |
| Jacket temperature.....    | 285° F.                                                       |
| Oil in temperature.....    | 185° F.                                                       |
| Oil out temperature.....   | 200° F.                                                       |
| Fuel.....                  | 100 octane (minimum) aviation type containing 4 ccs. TEL/gal. |
| Duration of run.....       | 50 hours                                                      |

In this test, electrical measurements are taken of the piston skirt deposit with respect to the extent or percentage of surface area of the piston skirt which is covered by the lacquer deposit at the termination of each run, together with the average thickness of the deposit expressed in inches  $\times 10^{-4}$ . Good reproducibility from run to run is obtained in the piston skirt lacquer deposit; and the test is therefore recognized as an accurate indication of the engine cleanliness of the oil composition under test.

The following results were obtained in this CFR High Speed Engine Test, utilizing the zinc alkyl phenolate preparations described above in conjunction with magnesium alkyl phenolate of known good quality in the proportions indicated, in a residual airplane engine oil having an SUS viscosity at 210° F. of about 120 and designated "AEO 120."

Table

| Zn Alkyl Phenolate Procedure     | Percent Conc. | Secondary Additive | Percent Conc. | CFR High Speed Engine Test Piston Skirt Deposit |                                 |
|----------------------------------|---------------|--------------------|---------------|-------------------------------------------------|---------------------------------|
|                                  |               |                    |               | Covered, Percent                                | Thickness, in. $\times 10^{-4}$ |
| 1. Example 1, ZP-24.....         | 0.5           | MP-24              | 1.0           | 32                                              | 0.17                            |
| 2. Example 2, ZP-23.....         | 0.5           | MP-23              | 1.0           | 37                                              | 0.53                            |
| 3. Example 3, ZP-21.....         | 0.5           | MP-23              | 1.0           | 39                                              | 0.19                            |
| 4. Example 4, ZP-23.....         | 0.5           | MP-23              | 1.0           | 21                                              | 0.08                            |
| 5. Example 5, ZP-23.....         | 0.5           | MP-23              | 1.0           | 0                                               | 0.00                            |
| 6. Example 5, ZP-23.....         | 0.5           | MP-23              | 1.0           | 8                                               | 0.01                            |
| 7. Example 6, ZP-23.....         | 0.5           | MP-23              | 1.0           | 0                                               | 0.00                            |
| 8. Standard ZP-21.....           | 0.5           | MP-21              | 1.0           | 0                                               | 0.00                            |
| 9. Standard ZP-21.....           | 0.5           | MP-21              | 1.0           | 0                                               | 0.00                            |
| 10. Base oil alone, AEO 120..... |               |                    |               | 80                                              | 2.0                             |

Run 10 of the foregoing table shows that the base oil alone fails to maintain engine cleanliness, since the piston was 80% covered with a comparatively thick lacquer deposit. On the other hand, a zinc alkyl phenolate of the proper quality in conjunction with magnesium alkyl phenolate of the proper quality, when employed in proportions of the order shown in the table, will maintain excellent engine cleanliness, and give in this engine test a piston substantially 10 without measurable lacquer deposit on the skirt.

Runs 1-4 inclusive of the table employed the zinc alkyl phenolate preparations of the foregoing Examples 1-4 respectively. While most of these products had ash and zinc contents fairly close to 15 theoretical, and some had fair solubility and storage stability, nevertheless the engine tests showed these products to be unsatisfactory as a detergent additive for the crankcase lubricating oil, since they failed to maintain the desired engine cleanliness. In the light of present knowledge, it appears evident that these earlier preparations failed because the required anhydrous conditions of reaction were not maintained, the proper long reaction time was not employed, the distillate 20 mineral lubricating oil was added prior to the reaction, and other procedural steps as enumerated above were not followed.

Runs 5 and 6 employed the two samples of the zinc alkyl phenolate produced in accordance with Example 5 above, wherein the standard procedure was employed except that the final refiltration in the presence of added light hydrocarbon solvent was not used. While the results of these runs showed very substantial improvement, Run 6 of the table gave a measurable lacquer deposit in the engine test.

Run 7 of the table employed the product made by the standard procedure of Example 6. Run 8 of the table employed a zinc alkyl phenolate preparation of different molecular weight which was also made by the standard procedure of Example 6. Run 9 of the table employed a zinc alkyl phenolate preparation made by the standard procedure, using in this case zinc chloride as the reactant in place of the zinc acetate of Example 6. As shown, these products were uniformly of excellent quality as detergent additives for the crank case lubricating oil. In addition to overcoming difficulties of filtration and purification of the product as encountered with the procedure of the prior art, the synthesis method of the present invention has been found to uniformly produce zinc alkyl phenolate products from these high molecular weight C<sub>15</sub>-C<sub>20</sub> alkyl phenols having the required solubility and stability in the residual airplane engine oil, and also the desired high quality as a detergent additive in maintaining excellent engine cleanliness.

Obviously many modifications and variations of the invention, as hereinbefore set forth, may be made without departing from the spirit and scope thereof and, therefore, only such limitations should be imposed as are indicated in the appended claims.

We claim:

1. In the manufacture of a zinc salt of an alkyl substituted hydroxy aromatic hydrocarbon consisting of carbon, hydrogen and oxygen, wherein the alkyl substituent on the ring contains from 15 to 30 carbon atoms, the improvement to obtain a zinc salt of at least 1% by weight solubility in a residual mineral lubricating oil of the airplane engine oil type and which has effective engine cleanliness properties, which comprises mixing under substantially anhydrous conditions and in the proportion of substantially one molar amount of an alkyl substituted hydroxy aromatic hydrocarbon consisting of carbon, hydrogen and oxygen, one molar amount of an alkali metal alcoholate of an aliphatic alcohol containing 4 to 6 carbon atoms in the molecule and boiling above the boiling point of water, said alkali metal alcoholate being in solution in an excess of the said anhydrous alcohol, and slightly more than one-half molar amount of a soluble zinc salt whose acidic portion forms an alkali metal salt which is insoluble in the said anhydrous alcohol, reacting the said mixture under refluxing conditions of the said C<sub>4</sub> to C<sub>6</sub> aliphatic alcohol for a period of time in excess of 20 hours to produce an anhydrous alcohol solution of the zinc salt of the alkyl substituted hydroxy aromatic hydrocarbon in which the alkali metal salt is precipitated, filtering to remove the precipitated alkali metal salt, adding to the filtrate a dry mineral lubricating oil, and stripping to remove the alcohol under anhydrous conditions to recover an anhydrous mineral lubricating oil concentrate of the said zinc salt having the aforementioned properties.

2. The method according to claim 1, wherein the alkyl substituted hydroxy aromatic hydrocarbon and the zinc salt are premixed, and the anhydrous C<sub>4</sub> to C<sub>6</sub> aliphatic alcohol solution of the alkali metal alcoholate is slowly added to the premixture at a lower temperature of the order of 30-70° C. and the resulting mixture is then raised to the alcohol refluxing temperature.

3. The method according to claim 2, wherein the said stripped mineral lubricating oil concentrate of the zinc salt is mixed with a dry light hydrocarbon solvent, the resulting mixture is re-filtered, and the light hydrocarbon solvent is then stripped from the filtered concentrate under anhydrous conditions.

4. The method according to claim 1, wherein the alkyl substituted hydroxy aromatic hydrocarbon is a C<sub>15</sub> to C<sub>20</sub> alkyl phenol, and the anhydrous C<sub>4</sub> to C<sub>6</sub> alcohol is a butyl alcohol.

JOHN W. HUTCHESON.  
EDWIN C. KNOWLES.

References Cited in the file of this patent

UNITED STATES PATENTS

| Number    | Name         | Date           |
|-----------|--------------|----------------|
| 2,197,833 | Reiff        | Apr. 23, 1940  |
| 2,399,877 | McNab et al. | May 7, 1946    |
| 2,610,982 | Hutcheson    | Sept. 16, 1952 |